

## UNITED STATES PATENT OFFICE

2,181,911

## PREPARATION OF NITROCELLULOSE

George A. Richter, Berlin, N. H., assignor to Brown  
Company, Berlin, N. H., a corporation of  
Maine

No Drawing. Application May 8, 1937,  
Serial No. 141,555

6 Claims. (Cl. 260—222)

This invention relates to the preparation of nitrocellulose and deals more particularly with treatments for improving cellulose fiber preparatory to its conversion into nitrocellulose.

5 In accordance with the present invention, cellulose fiber is nitrated in the form of paper fragments that have previously been treated with a chemical solution capable of inducing marked shrinkage therein upon their being dried, as they 10 are, preparatory to the nitrating reaction. There are various chemical solutions serviceable for the purposes hereof, including such reagents as strong aqueous solutions of sulphuric acid, zinc chloride, etc., which can cause partial gelatinization of 15 paper fragments and induce marked shrinkage therein when they are dried. However, a preferred reagent for the purposes hereof is caustic soda solution of mercerizing strength at the particular temperature at which it is applied to the 20 paper fragments, as a mercerizing solution not only induces the shrinkage or physical change desired in the paper fragments but also purifies the cellulose fiber of which such fragments are composed, thereby enabling the realization of high 25 grade nitrocellulose, whose quality is comparable to that realized from cotton, from paper fragments composed of wood pulp or other cellulose fiber with which is associated a significant percentage of non-alpha-cellulose constituents lend- 30 ing themselves to extraction or dissolution to a considerable degree in the mercerizing solution.

By reason of the marked shrinkage induced in paper fragments subjected to the treatments hereof preparatory to nitration, such fragments 35 are distinctly strengthened or toughened; and they hence do not tend to disintegrate during nitration into fine particles or shreds apt to be lost during the nitration or after-nitration treatments and thus conducing to lower than expected nitro- 40 cellulose yield. Indeed, the invention hereof enables the realization of excellent nitrocellulose yield even from paper fragments composed of low-viscosity cellulose fiber, which, by reason of treatment with dilute aqueous mineral acid solution, 45 oxidant solution or similar viscosity-reducing agent, has become sufficiently embrittled to impart tendency toward disintegration to paper formed from such fiber. By inducing marked shrinkage in such paper fragments and thereby 50 increasing their strength or toughness, disintegration thereof during the nitration and/or after-nitration treatments can be practically completely obviated. It might be noted that the marked shrinkage induced in the paper fragments 55 hereof is attended also by their curling or puck-

ering to such an extent that they do not tend to pack face to face in the nitrating bath; and this means both that the nitrating acid is given opportunity to diffuse rapidly and substantially uniformly into and throughout the bodies of the 5 fragments and that the acid is more readily and completely drained therefrom after nitration, especially when the so-called water-displacement method of draining the nitrating acid from the nitrated mass of fragments is employed and when 10 the water is similarly displaced by alcohol or equivalent dehydrating medium.

The practice hereof will now be described in terms of treatment of paper fragments with a mercerizing solution under conditions leading 15 to dried, mercerized fragments nitratable into so-called high-viscosity nitrocellulose. The paper sheet employed as starting material for such purpose is preferably composed of white, refined wood pulp of an alpha-cellulose content 20 upwards of about 93%, but, if desired, high grade bleached sulphite pulp and bleached kraft pulp may serve as the cellulose of such sheet. The paper sheet may be slit, as it is being progressively unwound from a roll, into 25 narrow strips or ribbons, for instance, of about  $\frac{1}{8}$  to  $\frac{1}{4}$  inch width, and the strips then cut transversely into paper fragments of, say, about 1 to 2 inches length. A mass of the resulting paper fragments may then be steeped in caustic 30 soda solution of about 16% to 20% strength at a temperature of about 15° to 20° C. If desired, the causticity of the solution may be as low as about 10%, provided that it is applied at sufficiently low 35 temperature to effect the desired marked mercerizing action on the paper fragments, say, at about 10° C. However, when a solution of a causticity even as low as about 10% is applied at too low a temperature, say, 5° C., it is quite difficult to maintain the integrity of the paper fragments by reason of the tendency of the fragments to disintegrate into a mush under the intense 40 swelling and mercerizing action thereupon of the solution at such low temperature. It is, accordingly, desirable to work with solutions having the 45 desired mercerizing activity under combined causticity and temperature conditions conducive to the maintenance without difficulty of the integrity of the paper fragments. The solution penetrates the mass and its individual fragments practically 50 instantly; and, after a soaking period of about 15 to 30 minutes, free caustic soda solution may be removed from the mass, as by centrifugation or equivalent treatment. Thus, the mass of solution-soaked fragments may be heated somewhat, for 55

instance, to a temperature of about 50° C., preparatory to its centrifugation so as to facilitate removal of solution therefrom. While the moist, centrifuged fragments are still in the centrifuge, 5 they may be washed with water, preferably heated to a temperature of, say, about 50° C., until practically no alkali residue remains therein, whereupon dilute sulphurous acid solution or its equivalent and wash water may be successively run into 10 the centrifuge in volumes sufficient to insure neutralization of residual traces of alkali and elimination of the products of neutralization. The finally washed and centrifuged mass of paper fragments may then be dried in any suitable way, 15 for instance, as in a hot-air chamber or tunnel, although it may be preferable in some cases to deliver air heated to a temperature of, say, about 100° C., into the centrifuge until the centrifuged mass is substantially completely dried.

20 The dried, mercerized fragments are of markedly smaller dimensions than the original fragments. Indeed, the shrinkage during drying may reduce the original area of the fragments by as much as about 10% to 20%, the particular reduction 25 in area depending upon the porosity or openness of structure of the original paper sheet. The dried fragments have a puckered appearance and a comparatively harsh feel, but they are very readily and substantially uniformly penetrated by 30 nitrating acid, water, and other reagents. When a mass of the fragments is nitrated with the usual mixed nitrating acid containing, say, about 24% nitric acid, at a temperature of about 30° to 40° C., a high nitrocellulose yield is had with low acid 35 retention. The nitrocellulose is of excellent quality and dissolves readily in the usual nitrocellulose solvents to form solutions of substantially perfect clarity. The nitrocellulose thus produced does not differ appreciably in viscosity from nitrocellulose prepared from the original or untreated 40 paper.

The inventive principles hereof are also applicable when so-called low-viscosity nitrocellulose is in view. For such purpose, the paper sheet may 45 be composed of cellulose pulp that has undergone bleaching or other treatment under conditions imparting thereto a viscosity of, say, about 0.4 to 4.0 poises, as measured by the standard method of producing and testing a cuprammonium-cellulose 50 solution. The paper may be cut into fragments, as already described; and a mass of the fragments may then be steeped in caustic soda solution of about 18% to 25% strength containing about 15% or more sodium hypochlorite bleach or equivalent 55 oxidant, based on the dry weight of paper, and at a temperature of about 45° to 60° C. After a soaking treatment of about two hours, when it is found that the viscosity of the cellulose has been reduced to about 0.1 poise, the mass of paper fragments 60 may be centrifuged, washed, and otherwise treated as previously described. Upon nitrating the resulting dried, mercerized paper fragments in the usual mixed nitrating acid but at a temperature of, say, 50° C., nitrocellulose of 12% nitrogen content is had; and such nitrocellulose dissolves in the usual nitrocellulose solvents to form 65 solutions of a viscosity comparable to those realized from the so-called half-second nitrocelluloses currently being marketed.

70 It might be noted that the preparation of low viscosity nitrocellulose might involve the use of cellulose pulp whose solution viscosity has been so markedly reduced by suitable chemical treatment prior to forming it into waterleaf paper that the 75 paper subsequently subjected to the processing

hereof in fragment form need be treated with mercerizing solution containing little, if any, oxidant to yield the desired low viscosity nitrocellulose. On the other hand, if the waterleaf paper has been formed from cellulose fiber of normal 5 solution viscosities, that is, from fiber which has not undergone a special chemical treatment designed to lower markedly its solution viscosity, the mercerizing solution subsequently applied to the paper in fragment form should, as indicated in the 10 example already given, contain an amount of oxidant capable of reducing the solution viscosity of the fiber to the low value desired.

It is possible to depart in various respects from the particular examples of procedure hereinbefore 15 described. Thus, the causticity and/or temperature of the mercerizing solution for treating the paper fragments may vary, but, in any event, the causticity and temperature of the solution are correlated so as to cause marked mercerization of 20 the cellulose fiber and thus induce the desired marked shrinkage in the paper fragments when they are dried. A caustic soda solution of about 15% to 25% strength may ordinarily be used to good advantage at a temperature of about 15° to 25 30° C., but the strength of the solution and/or the temperature at which it is applied may be higher or lower in instances when special characteristics are to be imparted to paper fragments. A time of treatment of about 30 minutes is usually all that 35 is necessary in the case of waterleaf paper of comparatively porous or open structure when the paper fragments being treated are to be converted into a high-viscosity nitrocellulose, but in those 40 cases when low-viscosity nitrocellulose is desired 45 and the treatment is conducted with a mercerizing solution containing an oxidant, the time of treatment should be extended to, say, two hours or even longer, and the solution is preferably heated to a temperature of, say, about 50° C. The 40 amount of oxidant added to the mercerizing solution is, as already indicated, also subject to variation, depending upon the particular viscosity desired in the nitrocellulose. On the other hand, 50 when high-viscosity nitrocellulose is being produced, it may be desirable to add to the mercerizing solution a suitable amount of sodium sulphide, sodium sulphite, or other reducing agent to minimize oxidative effect on the fiber and attendant reduction of its solution viscosity. Other secondary chemicals may be added to the mercerizing caustic soda solution. For instance, carbon bisulphide may be added thereto in very small 55 amount designed to increase swelling of the fiber and to enhance subsequent shrinkage of the paper fragments while avoiding such amount of carbon bisulphide as would cause sensible solution of fiber as cellulose xanthate.

Because the paper fragments are strengthened 60 or toughened by the mercerizing treatment hereof, they lend themselves to subsequent treatment without tendency to disintegrate into particles or shreds. Indeed, the mercerized paper fragments hereof may even undergo, preparatory to 65 nitrification, such treatments as bleaching, washing, neutralization with weak acid solution, another washing, and final dry. The dried fragments lend themselves nicely to storage and shipment in bale form.

70 The term "paper" as used in the foregoing description and in the appended claims is meant to include relatively thin waterleaf papers of a basis weight of, say, 30 to 50 pounds and thicker papers or boards, for instance, so-called pulp- 75

boards or drier sheets. The compactness of the paper or pulp sheets used herein may range from, say, about 60 to about 100. The compactness values given herein represent the ratio of basis weight to the sheet thickness in inches multiplied by the factor  $10^{-2}$ . The basis weight values given herein represent the weight in pounds of 415,000 square inches of sheet material. The term "fragments" as used herein is to be construed as meaning relatively small pieces of paper or pulpboard chips; and while elongated pieces or fragments of paper were described in the examples by reason of the fact that they can be baled and otherwise handled to good advantage, it is to be understood that the pieces or fragments might take the form of squares and other shapes.

It has been proposed in the prior art to nitrate paper after it has been conditioned by a method involving the passage of a progressively moving sheet through a bath of mercerizing solution, thence through a bath of wash water, and thence over drier drums or the like. In such a method, free shrinkage of the paper sheet is restrained and the paper sheet remains in contact with the mercerizing solution for only an exceedingly short period of time. The method hereof not only requires far less expensive equipment but makes possible far longer contact between the mercerizing solution and the paper and, accordingly, more pronounced mercerizing and purifying action on the paper; and, because the paper is mercerized and subsequently dried in fragment form and is under no restraint or tension during drying, it can shrink and pucker far more pronouncedly and thus, upon nitration, yield the improved results already indicated.

I claim:

1. A process of preparing nitrocellulose from cellulose fiber in the form of paper of a basis weight ranging from about 30 to about 100 pounds, which comprises cutting the paper into fragments of a minimum span in the order of magnitude of about  $\frac{1}{8}$  to  $\frac{1}{4}$  inch, treating a mass of such fragments with a mercerizing solution for a period of at least about fifteen minutes, washing the fragments substantially free from mercerizing solution, drying them, and nitrating the dried, mercerized fragments.
2. A process of preparing nitrocellulose from cellulose fiber in the form of paper of a basis weight ranging from about 30 to about 100 pounds, which comprises cutting the paper into fragments of a minimum span in the order of magnitude of about  $\frac{1}{8}$  to  $\frac{1}{4}$  inch, steeping a mass of such fragments in a mercerizing solution for a period of at least about fifteen minutes, removing free mercerizing solution from the resulting solution-soaked fragments, washing the fragments substantially free from the mercerizing solution,

drying them, and nitrating the dried, mercerized fragments.

3. A process of preparing nitrocellulose from cellulose fiber in the form of paper of a basis weight ranging from about 30 to about 100 pounds, which comprises cutting the paper into fragments of a minimum span in the order of magnitude of about  $\frac{1}{8}$  to  $\frac{1}{4}$  inch, treating a mass of such fragments with a mercerizing solution containing an oxidant for a period of at least about fifteen minutes, washing the fragments substantially free from such mercerizing solution, drying them, and nitrating the dried, mercerized fragments.

4. A process of preparing nitrocellulose from cellulose fiber in the form of paper of a basis weight ranging from about 30 to about 100 pounds, which comprises cutting the paper into fragments of a minimum span in the order of magnitude of about  $\frac{1}{8}$  to  $\frac{1}{4}$  inch, treating a mass of such fragments at elevated temperature with a mercerizing solution containing an oxidant of the nature of hypochlorite for a period of at least about fifteen minutes, washing the fragments substantially free from such mercerizing solution, drying them, and nitrating the dried, mercerized fragments.

5. A process of preparing nitrocellulose from cellulose fiber in the form of paper of a basis weight ranging from about 30 to about 100 pounds, which comprises cutting the paper into fragments of a minimum span in the order of magnitude of about  $\frac{1}{8}$  to  $\frac{1}{4}$  inch, treating a mass of such fragments with a chemical solution capable of effecting a gelatinizing action on cellulose fiber for a sufficient period of time to cause partial gelatinization of the fragments to such a degree that the fragments upon subsequent drying undergo at least 10% to 20% shrinkage in the area originally presented thereby, drying the fragments, and nitrating the dried, mercerized fragments.

6. A process of preparing nitrocellulose from cellulose fiber in the form of paper of a basis weight ranging from about 30 to about 100 pounds, which comprises cutting the paper into fragments of a minimum span in the order of magnitude of about  $\frac{1}{8}$  to  $\frac{1}{4}$  inch, treating a mass of such fragments with a chemical solution capable of effecting a gelatinizing action on cellulose fiber for a sufficient period of time to cause partial gelatinization of the fragments to such a degree that the fragments upon subsequent drying undergo at least 10% to 20% shrinkage in the area originally presented thereby, washing the partially gelatinized fragments substantially free from chemical solution, drying them, and nitrating the dried, mercerized fragments.

GEORGE A. RICHTER.